

W. A. SCHMIDT.

PROCESS FOR OBTAINING METALLIC VALUES FROM ORES.

APPLICATION FILED FEB. 2, 1920.

1,368,973.

Patented Feb. 15, 1921.



INVENTOR.

Walter August Schmidt

BY Arthur P. Knight

ATTORNEY.

# UNITED STATES PATENT OFFICE.

WALTER AUGUST SCHMIDT, OF LOS ANGELES, CALIFORNIA, ASSIGNOR TO INTERNATIONAL PRECIPITATION COMPANY, OF LOS ANGELES, CALIFORNIA, A CORPORATION OF CALIFORNIA.

## PROCESS FOR OBTAINING METALLIC VALUES FROM ORES.

1,368,973.

Specification of Letters Patent. Patented Feb. 15, 1921.

Original application filed April 29, 1918, Serial No. 231,459. Divided and this application filed February 2, 1920. Serial No. 355,818.

*To all whom it may concern:*

Be it known that I, WALTER AUGUST SCHMIDT, a citizen of the United States, residing at Los Angeles, in the county of Los Angeles and State of California, have invented a new and useful Process for Obtaining Metallic Values from Ores, of which the following is a specification.

This invention relates to the separation of minerals by volatilization, and particularly to the recovery from ores of copper, or other metals, of the chlorids of such metals by a volatilizing operation; this application being a division of my application Ser. No. 231,459, filed April 29th, 1918, for "Process for obtaining chlorids of potassium, or other metals."

In the volatilization of copper, or other metals, from ores thereof, it is usual to heat the ore in suitably divided condition, together with sodium chlorid, or other chloridizing agent, in such manner as to cause the production of the chlorid of the desired metal, such chlorid being then volatilized and the metallic fume collected in any suitable manner.

The main object of the present invention is to so carry out a process of this kind as to minimize the amount of sodium chlorid, or chloridizing agent, used and to provide for maximum efficiency of the volatilizing operation with such reduced amount of the chloridizing agent.

The accompanying drawing is a vertical section of a furnace suitable for carrying out the invention.

An important feature of the present invention is that the sodium chlorid, or chloridizing agent, is added to the finely divided ore during successive stages of heating thereof, whereby a given amount of chloridizing agent produces an increased volatilization of the metallic chlorid desired, or for any given amount of volatilization a reduced amount of chloridizing agent may be used.

My process is applicable to the recovery of any metallic chlorids more volatile than sodium chlorid, for example, it may be applied to volatilization of copper as chlorid from copper ores, the said ore being heated in the presence of sodium chlorid, or of sodium chlorid vapor, so as to form cupric chlorid which volatilizes and sodium sul-

fate, for example, which remains in the residue. The sodium chlorid is supplied continuously or intermittently, during the heating operation, so as to continue to supply sodium chlorid to the ore, as the copper chlorid is volatilized, until the required amount of copper content in the ore is driven off and collected, such collection being effected by electrical precipitation, by washing or otherwise. The heating operation may be carried on in a multiple hearth furnace, of the Herreshoff type, or the like, such as is shown at 1 in the drawing, the copper ore being fed in at the top hearth 2 by feeding means 3 and the sodium chlorid being fed in at several of the intermediate hearths 4, 5 and 6 by feeding means 7, 8 and 9. The sodium chlorid volatilized with the copper chlorid may be separated therefrom by solution and crystallization, or otherwise, and used in cyclic operation of the process. The volatilized chlorids are drawn from the upper part of the furnace to a suitable collecting means, either by the operation of natural draft, or by a suitable fan or blower.

The vapors resulting from heating the material with sodium chlorid in the manner above set forth, may be condensed by cooling in any suitable manner and the resulting product collected in any suitable collecting apparatus, preferably an electrical precipitator. In this connection the fact that a considerable quantity of hydrochloric acid is in some cases formed in the fuming operation tends to facilitate the deposition of the product in an electrical precipitator.

Silver ores and lead ores, or complex ores of silver, copper and lead may also be treated by this process, the amount of sodium chlorid added and temperature of volatilization being controlled in each case to produce the required volatilization. For silver chlorid volatilization a relatively high temperature will be required, and the furnace used must be such as to operate at such temperature. In such cases, a rotary kiln may be used. The chlorids volatilized from complex ores of silver, copper and lead may be condensed in stages by successive cooling operations, and the resulting condensed materials collected or precipitated at each stage, so as to effect more or less separation of such metals. In any case, it is desirable to

use more sodium chlorid than corresponds theoretically to the amount of copper, silver or lead, etc., as higher recoveries are thereby attained.

5 In some cases, other halids, for example, calcium chlorid, may be used instead of sodium chlorid, to increase the volatilization of potassium chlorid, it being understood that in this case the calcium salts may 10 remain mostly in the residue.

What I claim is:

1. The process of obtaining metallic chlorids from ores, which consists in subjecting the ore to heat and adding a metallic 15 chlorid to the ore at successive stages of the heating operation while the ore is maintained at sufficiently high temperature to effect chloridizing of the metallic content of the ores and volatilization of the resulting 20 chlorid.

2. The process of treating ores containing a metallic constituent in non-halid form

to obtain a halid of such metal, which consists in adding to such material a halid of another metal, heating the material, then 25 adding a further quantity of a halid of a metal other than the metal to be obtained as halids, and further heating the mixture to such temperature as to cause conversion of the said non-halid constituent to halid 30 form, and volatilization of the resulting halid.

3. The process of obtaining metallic values from ores, which consists in subjecting the ore to heat and adding a metallic 35 halid to the ore at successive stages of the operation under such temperature conditions as to effect conversion of the metallic content of the ore to halid form, and volatilization of the resulting halid.

In testimony whereof I have hereunto subscribed my name this 23rd day of January, 1920.

WALTER AUGUST SCHMIDT.